

## UNITED STATES PATENT OFFICE

PAUL VIRCK, OF DESSAU IN ANHEIM, GERMANY, ASSIGNOR TO GENERAL ANILINE WORKS, INC., OF NEW YORK, N. Y., A CORPORATION OF DELAWARE

## PROCESS OF DYEING PELTS, HAIRS, FEATHERS, AND THE LIKE

No Drawing. Application filed December 6, 1927, Serial No. 238,222, and in Germany September 14, 1926.

I have filed an application in Germany I, 29,039 IV/8m, filed Sept. 14, 1926; Austria: November 4th, 1927, Poland: filed November 9th, 1927.

This invention relates to a process of dyeing pelts, hairs, feathers or the like by means of naphthalene derivatives containing as substituent a 4-aminoarylaminogroup of the benzene series. The naphthalene residue 10 may also contain another substituent or substituents, for instance a hydroxy-, amino-, aminoarylaminogroup.

The compounds used according to my invention correspond to the general formula:



20 wherein X means hydrogen or a univalent substituent such as alkyl or halogen and wherein Y means H, —OH, —NH<sub>2</sub>, —NH—aryl—NH<sub>2</sub> or halogen.

The mordanted or not mordanted goods 25 are treated with an aqueous solution of a salt of such a 4-amino-aryl-amino-derivative of the naphthalene and then with a suitable oxidizing agent; there are thus produced fast red-violet to black-blue and greenish grey 30 tints.

The following examples illustrate the invention:

Example 1.—In a bath containing per liter 2 grams of 2-(4'-aminophenylamino)-naphthalene hydrochloride, some alcohol and a quite small proportion of hydrochloric acid, a thoroughly killed and, if necessary, mordanted skin is handled at the ordinary temperature for some hours. The skin is then 40 washed and treated for one hour in a separate bath containing per liter 20 grams of potassium bichromate and 20 grams of acetic acid of 30 per cent strength. There is obtained a blue-green dyeing.

45 A skin which has been thus mordanted

with potassium bichromate is dyed bluer when it is subjected to the first treatment prescribed in Example 1 and then to a subsequent treatment with hydrogen peroxide in ammoniacal solution; when the preliminary mordant is a copper compound a black-blue dyeing is produced.

50 Red-violet to currant tints are obtainable when 1-(4'-aminophenylamino)-naphthalene is used under the conditions named in Example 1.

55 Example 2.—A thoroughly killed and, if necessary, mordanted skin is handled in a bath containing per liter 5 grams of 2-(4'-aminophenylamino)-6-hydroxynaphthalene hydrochloride, some alcohol and a small proportion of hydrochloric acid for some hours at ordinary temperature. After washing, the skin is treated with an oxidizing agent. When the latter is an acidified solution of 60 bichromate a dark green-blue grey tint is obtained.

65 With 2-(4'-aminophenylamino)-6-(4'-aminophenylamino)-naphthalene there is obtained a similar rather more greenish-grey tint; 1-(4'-aminophenylamino)-5-(4'-aminophenylamino)-naphthalene yields violet grey dyeings when the subsequent treatment is with a solution of alkali bichromate and acetic acid. 1-(4'-aminophenylamino)-5-hydroxynaphthalene yields under like conditions a blue-violet, 2-(4'-aminophenylamino)-7-hydroxynaphthalene a bluish violet, 2-(4'-aminophenylamino)-7-(4'-aminophenylamino)-naphthalene a violet grey tint which 70 by prolonged treatment with bichromate and acetic acid becomes violet or bluish.

75 When the phenyl group contains a substituent such as alkyl or halogen, the applicability of the naphthalene derivative is 80 not affected.

85 What I claim is:

1. A process of dyeing pelts, hairs and feathers, by successively treating the goods 90

with an aqueous solution of a salt of a naphthalene derivative of the general formula:



(wherein X means H or an univalent substituent of the group consisting of alkyl and halogen and wherein Y means H or an univalent substituent of the group consisting of —OH, —NH<sub>2</sub>, —NH—aryl—NH<sub>2</sub> and halogen) and with an oxidizing agent.

2. A process of dyeing pelts, hairs and feathers, by successively treating the mordanted goods with an aqueous solution of a salt of a naphthalene derivative of the general formula:



(wherein X means H or an univalent substituent of the group consisting of alkyl and halogen and wherein Y means H or an univalent substituent of the groups consisting of —OH, —NH<sub>2</sub>, —NH—aryl—NH<sub>2</sub> and halogen) and with an oxidizing agent.

30 3. A process of dyeing pelts, hairs and feathers, by successively treating the goods with an aqueous solution of a salt of a naphthalene derivative of the general formula:



(m being a whole number not less than 1 and not greater than 2) and with an oxidizing agent.

40 4. A process of dyeing pelts, hairs and feathers, by successively treating the mordanted goods with an aqueous solution of a salt of a naphthalene derivative of the general formula:



(m being a whole number not less than 1 and not greater than 2) and with an oxidizing agent.

50 5. A process of dyeing pelts, hairs and feathers, by successively treating the goods with an aqueous solution of a salt of a naphthalene derivative of the general formula:



and an oxidizing agent.

60 6. A process of dyeing pelts, hairs and feathers, by successively treating the mordanted goods with an aqueous solution of a salt of a naphthalene derivative of the general formula:



and an oxidizing agent.

7. A process of dyeing pelts, hairs and feathers, by successively treating the goods with an aqueous solution of 2-(4'-aminophenylamino)-naphthalene hydrochloride and an oxidizing agent.

8. A process of dyeing pelts, hairs and feathers, by successively treating the mordanted goods with an aqueous solution of 2-(4'-aminophenylamino)-naphthalene hydrochloride and an oxidizing agent.

In testimony whereof, I affix my signature.

PAUL VIRCK.

70

75

80

85

90

95

100

105

115

110

120

125

130